

Sept. 6, 1927.

1,641,478

D. FINLEY

## PROCESS OF TREATING PAPER

Filed Sept. 6, 1922



WITNESS  
*H. G. Sherburne,*

INVENTOR  
DOZIER FINLEY.  
BY White Bros. & Evans

his ATTORNEYS

Patented Sept. 6, 1927.

1,641,478

# UNITED STATES PATENT OFFICE.

DOZIER FINLEY, OF BERKELEY, CALIFORNIA, ASSIGNOR TO THE PARAFFINE COMPANIES, INC., OF SAN FRANCISCO, CALIFORNIA, A CORPORATION OF DELAWARE.

## PROCESS OF TREATING PAPER.

Application filed September 6, 1923. Serial No. 586,441.

My invention relates to paper and a process of incorporating crystalline material in the paper during its manufacture.

An object of the invention is to provide a process for depositing or incorporating crystalline material in the sheet of fiber during the course of its manufacture and preferably, after a portion of the water has been drained from the wet sheet while it is on the 10 wire or carrier felt, at some stage before the sheet has passed thru the press rolls.

Another object of the invention is to provide a paper in which a quantity of crystalline material has been included so that the 15 strength, weight and porosity of the sheet are increased, and qualities imparted which are characteristic of the material used.

My invention possesses other objects and features of advantage, some of which, with 20 the foregoing, will be set forth in the following description of my invention. It is to be understood that I do not limit myself to the showing made by the said description, as I may adopt variant forms of my invention 25 within the scope of the claims.

Referring to the drawings: Fig. 1 is an elevation in diagram of an apparatus with 30 which the process of my invention may be performed. Fig. 2 is a similar view of a modified form of such apparatus. Fig. 3 is an elevation in diagram of a portion of another apparatus with which the process of 35 my invention may be performed in connection with the manufacture of paper board.

In the following specification, I shall use 40 the term "paper" in a generic sense to include all fibrous sheets in which the process of manufacture comprises the conversion of a mass of fiber suspended in liquid, into a sheet or layer, or a plurality of constituent sheets or layers, from which the water is afterward expressed by squeezing and drying; and this term includes not only paper in 45 the restricted and specific meaning, but also paper board and felt.

Papers are possessed of certain qualities 50 or characteristics common to all, and other qualities or characteristics peculiar to particular kinds of papers. The most important 55 of these qualities which all papers must possess is strength, and each kind must have a strength requisite to its intended use. Thickness is another important character- 60 istic which must be such as to adapt the

paper for its purpose. Porosity is a quality 55 of the highest importance in felt, since most of the felt manufactured is saturated with asphaltic compounds. Resistance to fire and decay, and germicidal properties are other characteristics of importance. By the practice of my invention I am enabled to vary the degree of these qualities, so that the resultant product discloses an enhanced value and intensified or increased adaptability for its intended use. 65

Referring to Fig. 1, which illustrates a felt making apparatus, an endless wet or carrier felt belt 2 is arranged in a well known manner upon idler rolls 3, couch roll 4 and between press rolls 6. A screen cylinder 7 is 70 disposed below the couch roll, and a drying drum 8 is arranged to receive the wet formed sheet of felt 9 which, first forming on the screen cylinder, is picked up by the carrier felt and passed thru the press rolls to express the excess of fluid. 75

Arranged above the formed felt sheet preferably just after it leaves the couch roll is a rotatable spindle 12 provided with vanes 13. A tank 14 is disposed above the spindle and a perforated valve controlled pipe 15 permits solution from the tank to fall in regulatable quantities upon the revolving vanes, which break up the flow and evenly distribute the solution over the surface of the 85 sheet in the form of a fine spray, which is instantly absorbed by the formed sheet as it passes below.

The fluid in the tank 14 is preferably an aqueous solution of sodium chloride containing about 26% by weight of the salt, but for certain purposes which will be made clear later, other water soluble crystalline material may be substituted. 90

Between the vanes and the press rolls and 95 below the carrier felt is a suction box 17 for abstracting a portion of the liquid from the formed sheet and the carrier felt. The salt solution discharging from the revolving vanes, tends to work downwardly in the 100 formed sheet, gravitation, the suction box and the press rolls, all helping the salt solution to displace the water present in the sheet as it leaves the couch roll. The suction box will remove the water on the lower side of the sheet and in the carrier felt, and as the first water is taken out, the salt solution sinks further into the formed sheet. If a 105

carefully regulated amount of salt solution is applied to the formed sheet, it will just penetrate to the under side of the sheet by the time the press rolls have been passed.

5 The sheet, after drying on the cylinder 8, is found to be heavily charged with salt, and as an illustration of the results obtained by the application of a salt solution on a fiber sheet in its process of manufacture on a felt 10 making machine the following results are given: Comparisons are made with a similar sheet, untreated, and manufactured under ordinary well known manufacturing conditions; both sheets being of the same weight, 15 thickness, and strength before the treatment of one of them.

|                                              | Untreated sheet | Treated sheet |
|----------------------------------------------|-----------------|---------------|
| 20 Weight.....                               | grams.....      | 9.95          |
| Thickness.....                               | inches.....     | .0384         |
| Strength per square inch by Mullen test..... | pounds.....     | 16.5 21       |

25 From this it is seen that a stronger, heavier and slightly thicker product is obtained. The sheet treated with salt solution was tested for porosity by weighing it and saturating it in an asphaltic compound. It was then compared to a companion sheet from which it differed only in having undergone treatment with the salt solution.

|                                               | Untreated sheet | Treated sheet |          |       |          |
|-----------------------------------------------|-----------------|---------------|----------|-------|----------|
|                                               |                 | Grams         | Per cent | Grams | Per cent |
| 35 Felt fiber present.....                    | 17.7            | 48.9          |          | 17.7  | 39.8     |
| Soluble salts added by treatment.....         |                 |               |          | 5.1   | 11.4     |
| Asphaltic compound necessary to saturate..... | 18.5            | 51.1          |          | 21.7  | 48.8     |
| 40                                            | 36.2            | 100.0         |          | 44.5  | 100.0    |

It will thus be seen that in the treated sheet there is not alone a total of 11.4% of the cheaper mineral salt, but in the treated 45 sheet, the ratio of felt fiber to asphaltic compound is 1 to 1.226 whereas in the untreated sample such ratio is 1 to 1.045. The actual percentages of saturation, based on the weights of fiber and asphaltic compound are 50 122.6 for the treated, and 104.5 for the untreated test sheets, although the apparent saturation of the treated sheet is but 95.3%. The saturated untreated sheet gave a Mullen test of 42.75 pounds, the saturated treated 55 sheet 48.5 pounds.

The results of the above tests clearly demonstrate that for a given weight of paper or felt which is to be saturated, my process will permit a smaller quantity of the more valuable fibrous ingredients to be used, the difference being supplied by a corresponding increase in the cheaper soluble salts incorporated. That is to say, my process involves the use of a certain amount of sodium chloride or such other crystalline material of a

relatively high degree of solubility in water and the cost of which is below that of the corresponding amounts of paper making fiber which it displaces.

Sodium chloride is preferably employed 70 in my process, because it is more abundant and cheaper than any other suitable crystalline material; it does not absorb moisture to an appreciable extent when dried; it is readily mixed in solution of the desired concentration; it is not readily decomposed by heat; and it is non-poisonous and does not react with other normally occurring substances to produce poisonous or unstable compounds. When deposited in the paper from water solution it forms desirably shaped crystals incrusted upon the fibers, pushing them apart somewhat to produce a greater degree of porosity, and at the same time interlocking the fibers so that the strength of the sheet is materially increased.

Although I prefer sodium chloride for the reasons named, I may use other materials, such as magnesium sulphate, sodium borate, or disodium hydrogen phosphate. Mixtures of salts may be used, as for example, a small amount of calcium chloride, or magnesium chloride in conjunction with the sodium chloride. Both calcium and magnesium chloride take up moisture from the air, and by their use, a degree of softness is imparted to the treated sheet. I contemplate also, the use of a salt such as ammonium phosphate or ammonium sulphate to render the sheet fire resistant; or a salt such as zinc sulphate to impart germicidal properties, and prevent decay both in the sheet itself and the surface on which it lies. In this connection, copper acetate is also good, but the use of copper in any of its forms on a machine composed 100 largely of the ferrous metals is undesirable since the copper is readily ionized if water is present, and in that form, quickly eats away all ferrous parts with which it establishes an electrolytic relation. For this reason zinc 110 sulphate is superior to a copper salt, and it does not react on the paper fiber as does copper sulphate which liberates free acid.

While I have so far mentioned only mineral salts, it is possible to use salts of the 115 organic acids combined with mineral bases, or combined with organic bases, or crystalline organic materials other than organic salts or esters to accomplish the purposes of my process. For example, one of the sugars 120 may be used.

In Fig. 2, I show an apparatus for applying the salt in another way. A box 19 having a 100-mesh screen bottom is arranged above the formed sheet, and provided with 125 well known means for shaking it. A quantity of water soluble crystalline material finely pulverized is placed in the box and as the formed wet sheet passes below the shaking box, the material is evenly sprin- 130

kled upon it and is quickly dissolved by the water in the sheet. By the time the sheet has passed the press rolls, the solution has worked thru it in the manner already made 5 clear.

A type of apparatus for making paper board is illustrated in part in Fig. 3, in which the component sheets of fiber are formed on cylinders 21 and taken off by the 10 carrier belt 22, which passes over suction box 23 and between small press rolls 24 and large rolls 25. In this case a "top felt" 27 passes thru the press rolls in contact with the upper surface of the formed sheet. At 15 a convenient point, the top felt is washed by a spray 28 of fresh water and mechanically whipped by a whipper 29.

To prevent the top felt absorbing any considerable quantity of salt solution from 20 the formed sheet of board, a relatively light shower of water is sprinkled on the sheet by means 31 which may be similar to the solution spreading means already described. The effect of this shower of water is to drive 25 down the salt solution previously applied so that the salt solution is capped by a layer of fresh water. The subsequent operations of expressing liquid from the board sheet in an upward direction into the top felt, will 30 proceed only so far as to remove this layer of fresh water. Of course some salt solution will be absorbed into the top felt, but most of this may be recovered by spraying the upper reach of the top felt with fresh 35 water from a pipe 32 just before the felt passes over a suction box 33. The fresh water will be drawn out by the suction box carrying with it most of the salt solution. This recovered dilute solution may be used

in preparing the concentrated solution for 40 the tank 14.

I claim:

1. The process of treating a formed wet sheet of paper which comprises displacing water normally present therein with an 45 aqueous solution of a sodium chloride.

2. The process of treating a formed wet sheet of paper which comprises flowing a solution of crystalline material upon the surface of the wet sheet, subjecting the opposite 50 surface to a vacuum to displace the water normally present in the sheet with the solution, and evaporating the water to crystallize the material upon the fibers with interlocking effect. 55

3. The process of treating a formed wet sheet of paper which comprises flowing a solution of sodium chloride upon the surface of the wet sheet, subjecting the opposite 60 surface to a vacuum to displace the water normally present in the sheet with the solution, and evaporating the water to crystallize the salt upon the fibers with interlocking effect.

4. The process of treating a formed wet sheet of paper which comprises flowing upon the entire surface of the sheet a solution of crystalline material in quantity sufficient to substantially equal the water normally present in the sheet, subjecting the opposite 70 surface to a vacuum to displace the water normally present in the sheet with the added solution, and evaporating the free liquid from the sheet to incrust the fibers with the crystalline material. 75

In testimony whereof, I have hereunto set my hand.

DOZIER FINLEY.